

(No Model.)

H. T. SMITH.

MANUFACTURE OF HOLLOW PLATED METAL INGOTS AND  
SEAMLESS WIRE.

No. 432,496.

Patented July 15, 1890.



FIG. 1.



FIG. 3.



FIG. 2.



FIG. 4.



FIG. 5.

WITNESSES:

*George M. Cady.*  
*W. W. Jones*

INVENTOR:

*Henry T. Smith*  
by *Edson Salisbury Jones*  
Attorney

# UNITED STATES PATENT OFFICE.

HENRY T. SMITH, OF PROVIDENCE, RHODE ISLAND, ASSIGNOR, BY DIRECT AND MESNE ASSIGNMENTS, TO ROSWELL C. SMITH, TRUSTEE, OF SAME PLACE.

## MANUFACTURE OF HOLLOW PLATED-METAL INGOTS AND SEAMLESS WIRE.

### SPECIFICATION forming part of Letters Patent No. 432,496, dated July 15, 1890.

Application filed April 18, 1890. Serial No. 348,540. (No specimens.)

*To all whom it may concern:*

Be it known that I, HENRY T. SMITH, of the city and county of Providence, and State of Rhode Island, have invented certain new and useful Improvements in the Manufacture of Hollow Plated-Metal Ingots and Seamless Wire Therefrom; and I do hereby declare the following specification, taken in connection with the accompanying drawings forming a part of the same, to be a description thereof.

This invention relates to a process of producing hollow plated-metal ingots and seamless wire therefrom for the use of jewelers, &c.

In Letters Patent of the United States issued to me March 4, 1890, and numbered 422,647, there is described a process of forming a tubular-shaped ingot from a circular compound plate of metal, which process consists in drawing up such plate, by means of suitable dies and plungers, into the form of a tube having a closed end. When the circular compound plate or rudimentary ingot is comparatively thin, no trouble is experienced in producing the tubular ingot without imperfections, provided a suitable number of dies and plungers be used in the drawing-up process. When, however, seamless plated wire is to be manufactured on a large scale and of great length, the compound plate or rudimentary ingot must be quite thick, and a large number of dies and plungers would be necessary to draw up such plate into tubular form. Experience has shown me that even when a very large number of dies and plungers are employed and great care is exercised the gold or other superior metal forming the outer portion of the ingot will crack in some places during the drawing up of the compound plate into tubular form, owing to the thickness of the plate or rudimentary ingot and the tendency of the superior outer portion thereof to "crawl" or separate under great strain and the friction of such superior outer portion of the ingot against the walls of the dies. These cracks in the superior metal of the ingot become enlarged when the ingot is reduced or drawn into wire, thereby rendering the wire imperfect.

To obviate the crawling or cracking of the superior outer portion of the ingot during the

formation of it into a tube is the object of the present invention, and this is accomplished as hereinafter described and claimed.

The better to illustrate my improved process there is shown in Figure 1 of the drawings a rudimentary compound ingot in perspective, the shape of said ingot being that of a circular plate. Fig. 2 shows this rudimentary ingot drawn up into cup form. Fig. 3 represents the same reduced in diameter and elongated into tubular form. Fig. 4 shows a small piece of seamless plated wire produced from such tube. Fig. 5 represents in perspective a pair of dies for use in trip-hammering the cup-formed ingot into the tubular form shown in Fig. 3.

A represents the rudimentary ingot, which is preferably in the form of a circular plate, one portion *a* of which is composed of copper or other suitable low-grade metal, and the other portion *a'* of gold or other superior metal soldered or otherwise secured to one of the faces or sides of the plate *a*. By means of one or more properly-shaped plungers and dies the compound plate *A* is drawn or stamped up into the form of a cup *B*, the gold or superior metal portion of the compound plate being upon the outside. Experience has shown that such a rudimentary ingot five-sixteenths of an inch thick can be drawn or stamped up into the cup form *B* by one or more suitable dies and plungers without producing any cracks in the superior outer portion of the ingot.

To reduce the cup-shaped ingot *B* to the tubular form *C*, I employ a trip-hammer and several pairs of duplicate dies, as *D*, one die of each pair being preferably located on a stationary bed and the other being secured to the hammer-arm or head. Preferably the walls of these dies taper, as shown at *d*, Fig. 5, and terminate at one end in a groove whose walls *d'* are parallel. By means of a suitable number of such duplicate dies the cup-shaped ingot *B* may be trip-hammered, and thereby reduced in diameter and elongated to the form of the tube *C*, and this elongation and reduction of size may be continued until the diameter of the tube has been greatly reduced, if desired, without any danger of the superior

metal forming the outer portion of the ingot being cracked, for the trip-hammering absolutely preserves the integrity of the superior outer portion of the ingot. Not only does this trip-hammering preserve the integrity of the superior outer metal of the ingot, but the reduction of the cup-formed ingot to a tube or even to a rod can be accomplished in much less time and with very many less dies or tools, besides requiring many less annealings than would be necessary were not such trip-hammering employed in the process of reduction.

If, for example, the compound plate or rudimentary ingot A be six inches in diameter and five-sixteenths of an inch thick, such plate may be drawn or stamped up by a single die and plunger into the cup form B, which will be about four inches in diameter and two and one-fourth inches deep, without cracking the superior outer portion of the ingot. This cup-formed ingot is then subjected to the action of several pairs of duplicate dies in a trip-hammering machine, and if three pairs of such dies be used the ingot may be reduced to the tube form shown in Fig. 3, which will be about one and one-fourth inch in diameter and seven inches long. This tube-formed ingot may then be operated upon by well-known reducing machinery to fit it for the "draw-bench." If desired, however, the trip-hammering of the ingot may be continued by proper dies until it has been reduced sufficiently in diameter to be operated upon in a draw-bench.

35 By means of a draw-bench or rolling-machine the ingot may be drawn into wire of any desired gage or diameter, and if it be reduced to size No. 27, Brown & Sharpe gage, a coil of seamless plated wire about four thousand four hundred (4,400) feet long will be produced, the outer or superior portion of which will be free from cracks or flaws.

From the foregoing it will be readily understood that the rudimentary ingot A can be formed into the cup B by a single die and plunger, and such cup can be reduced by

trip-hammering with a few dies to a diameter suitable to be operated upon in a draw-bench, thus saving a great deal of time, many dies and tools, and many annealings, as well as obviating all cracking of the superior outer portion of the ingot. 50

What I claim, and desire to secure by Letters Patent, is—

1. The improvement in the process of forming hollow plated-metal ingots, which consists in drawing or stamping up a compound plate into cup form with the superior metal on the outside, then trip-hammering such cup into a tube form by means of dies, substantially as set forth. 55

2. The improvement in the process of forming seamless plated wire, which consists in drawing or stamping up a compound plate of metal into cup form with the superior metal on the outside, then trip-hammering such cup into a tube or rod, and finally drawing or reducing such tube or rod into wire, substantially as set forth. 60

3. The improvement in the process of forming seamless plated wire from a cup-formed ingot having the superior metal on the outside, which consists in trip-hammering such cup-formed ingot between dies to reduce it into a tubular or rod form, and finally drawing or reducing such tube or rod into wire, substantially as set forth. 70

4. The improvement in the process of forming seamless plated wire, which consists in soldering or attaching a plate of superior metal to a plate of low-grade metal, drawing or stamping up such compound plate into a cup-formed ingot, trip-hammering such cup-formed ingot into a tube or rod by means of suitable dies, and finally drawing or reducing such tube or rod into wire, substantially as set forth. 80

HENRY T. SMITH.

Witnesses:

EDSON SALISBURY JONES,  
M. W. JONES.